

Oct. 9, 1951

J. BAUER

2,570,750

BRASHENING OF WOOL

Filed Oct. 21, 1948

*Fig. 1.*



*Fig. 2.*



INVENTOR

*Jackson Bauer.*

BY

*Wm. S. Jackson & Son*

ATTORNEYS.

## UNITED STATES PATENT OFFICE

2,570,750

## BRASHENING OF WOOL

Jackson Bauer, Newportville, Pa., assignor to Fred Whitaker Company, a corporation of Pennsylvania

Application October 21, 1948, Serial No. 55,765

8 Claims. (Cl. 117—141)

1

The present invention relates to the treatment of wool and to wool pile fabrics produced by such treatment.

A purpose of the invention is to impart to wool the characteristics associated with brashness, and thus to permit the conversion of non-brash South American wools into brash wools as required, and to enhance the brashness of wool having some brashness.

A further purpose is to increase the wear resistance of woolen pile fabric such as upholstery, carpets and rugs. A further purpose is to obtain greater wiriness, or stiffness combined with resilience, in wool.

A further purpose is to create or enhance artificially the characteristics associated with brashness in wool and to secure a high degree of permanence in such treatment, which will even resist several hours of boiling, as well as normal dyeing, spinning, lubricating, weaving and subsequent laundering of the fabric.

A further purpose is to apply silica sol on the acid side under conditions which tend to agglomerate the sol and form gel, but without exhausting the solution by precipitation and to introduce such gross silica agglomerates to and in the wool.

A further purpose is to avoid the presence of oil especially as oil emulsion during the treatment.

A further purpose is to carry on the treatment in a normal wool treating solution such as a bleach.

A further purpose is to aid the application optionally by including of a dispersing agent, a substantive agent or an impregnating resin.

Further purposes appear in the specification and in the claims.

In the drawings I have chosen to illustrate one only of numerous embodiments in which the invention may appear, choosing the form shown from the standpoints of convenience in illustration, satisfactory operation and clear demonstration of the principles involved.

Figure 1 is a diagrammatic cross section of a woolen pile fabric of the character to which the invention is applied.

Figure 2 is a curve useful in explaining the invention.

In the prior art, colloidal silica sols in water solution have been used for reducing the slippage and increasing the tensile strength of textile fibers including wool. The procedure followed has generally been to apply such sols to the wool with the oil emulsion in the picker.

Colloidal silica sols can be made in various ways and the detail of production of the sols forms no part of the present invention. For example, finely divided silica can be put through a colloid mill with water and converted to a silica sol. The particle size of the silica for this purpose usually is in the range between 10 and 50 millimicrons. Likewise, the sols can be made chemically as for example according to the proc-

2

ess of any of the following U. S. patents: White, No. 2,375,739; Bird, No. 2,244,325; Powers et al., No. 2,443,512; Marshall, No. 2,285,449; and White, No. 2,285,477. The particle size of this chemically prepared material is usually of the order of 20 to 60 or 40 to 80 millimicrons, and for the present purpose the silica sol may vary from 10 to 100 millimicrons initially, but the smaller silica particles in order to become effective will be greatly increased in size during the treatment as explained below. The silica of the sol will in many cases be hydrated by the method of preparation used.

In the prior art treatment of textiles with silica sols, the effort has been to improve spinability and to increase tensile strength. The treatment has been very fugitive, and one of the advantages urged for the prior art wool treatment has been that it is completely removed from the fiber or cloth by a mild wash.

The present invention is concerned with a wholly different purpose from the improvement of spinability or tensile strength. It has been recognized for many years that satisfactory production of woolen pile fabrics such as carpets and upholstery requires the use of a wool having certain characteristics.

The wool must remain upright in the pile yarn and the pile fabric made from such yarn should possess the property of restoring itself to its original upright position after it has been depressed. The combination of characteristics which are generally known in the trade to be required in a carpet wool is herein referred to as "brashness," and a wool having such characteristics is herein referred to as "brash" or "brashy." For the purpose of this application the characteristics which produce brashness are defined as a combination of those characteristics exhibited in carpet wool which are described as coarseness, roughness, harshness, stiffness, hairiness, and wiriness, combined with the requisite resilience and resistance to deformation or stress.

The exact cause of the condition of brashness is apparently not fully known, since two wools may have the same fiber cross sections and other observable physical characteristics, and yet one wool will be generally suited for carpet wool purposes while the other will not. Thus there are large quantities of South American wools which are of suitable fiber cross section for use in the best pile fabrics, but which are precluded from general use for such purpose because of lack of brashness. There are also wools which have only slight brashness and can only be used to small extents in brash blends.

The same characteristics which are above discussed in reference to pile fabrics are useful also in other fabrics, wherever a brashy wool is required.

I have discovered that the characteristics associated with brashness can be imparted artificially to wool or artificially enhanced and that

unlike the previous treatments intended to aid spinability, brashness can be permanently imparted so that the wool will remain brash throughout the process and after subsequent laundering of the fabric. I have also discovered that by the same treatment the wear resistance of the pile can be tremendously increased.

Thus in accordance with the invention a South American or other non-brash wool can be converted permanently into a wool which exhibits the desirable characteristics of the better grades of carpet wool. Thus wools which previously had been considered "soft" for their particular fiber size and accordingly have been known as blanket or clothing wools, can be converted completely into wools suitable for carpet and upholstery use.

The effect of the treatment will be substantially resistant to several hours of boiling in water, and to the normal dyeing, spinning, lubricating, weaving and laundering operations, so that it can be applied at an early stage in the processing of the wool. It is not, however, practical to apply it in the picker with the oil emulsion, as the desired brashness is not acquired and the slight results obtained are not permanent.

It is of incidental but considerable benefit that the treatment likewise serves to deluster the wool, thus avoiding the necessity of separate delustering where required.

I have discovered that it is not possible to obtain permanence in the treatment unless the wool is previously degreased to a total grease content of less than 1.5% and preferably less than 3/4% before treatment. The percentage is based on the dry weight of the wool. If the wool is treated in the grease, I find that the treatment is not permanent and is otherwise unsuitable. The grease content should normally run between 1 and 3/5% after scouring and before treatment with silica, and I prefer to scour to a total grease content of 1/2% or less. In any case, other factors involved being equal, as the grease content increases, the effectiveness of the treatment decreases. Whenever grease content is referred to herein, it is intended to designate grease content as measured upon extraction by carbon tetrachloride at room temperature. Where degreasing is referred to it is intended to include solvent scouring as well as soap or detergent scouring.

I have also discovered that the remarkable results obtained by the present invention are not produced unless the operations are performed under acid conditions. The acidity may be imparted in either of two ways, either as acidity in the treating solution or acidity previously imparted to the wool.

Without limiting myself to the theory herein set forth, my experiments indicate that the effect of acidity is to cause the particles of silica sol to agglomerate and produce gross particles which enter into the wool fiber forming a silica matrix, and also to some extent deposit on the fiber. I believe that the scouring or degreasing to the extent indicated is necessary to permit penetration through the epidermis of the fiber, so that a network or matrix of silica can build up in the cortical layer or the medulla, either in the porous air channels which are there present or in or among the cells or fibrils. A further reason for removing grease is that the presence of a grease film in or on the fiber may prevent such bonding between the wool and the silica as may be the result of the existence of opposite electrical charges on the wool and the silica. My experiments indicate that the improved properties are

not due to increase in external diameter, but are due to action primarily within the fiber or on the surface but in such amounts as not to affect fiber diameter.

5 The extreme firmness of adhesion obtained suggests that the disposition of the silica is not purely physical but involves the operation of secondary valences, and is therefore also chemical.

#### Example I

A control was used for comparison with the treated sample which consisted of a high grade India carpet wool. The sample to be treated was a South American wool having the same approximate fiber size as the control, but initially having a comparatively soft feel, and known in the trade as a blanket wool or clothing wool. The wool to be treated was scoured in the ordinary manner to a total grease content of 0.3%. The degreased wool was then treated continuously in a full size standard wool bowl, with a solution consisting of water containing 0.6% of silica sol made by diluting commercial silica sol dispersion with water to the concentration mentioned. The solution also contained 0.1% of sulphuric acid. The solution was free from oil.

The wool was passed through the bowl under ordinary conditions, at a rate which assured exposure to the solution for about 1 1/2 minutes.

30 The temperature of the solution was 115° F.

Under these conditions, in the presence of the normal impurities brought into the solution by the wool, the particles of silica agglomerated, and a small amount of precipitate formed as the impurities carried in with the wool acted on the solution. This is not objectionable. The wool picked up silica in proportion to the pick-up of solution, which was controlled by squeeze rolls at the end of the bowl.

40 After passing through the treating bath, and squeezing to remove excess treating liquid, the wool, when inspected in the wet, showed little evidence of change in brashness. The wool was then carried through a standard wool drier and brought to equilibrium with the atmosphere of the room. After the moisture content had reached equilibrium with the atmosphere at about 12%, the treated wool was compared with the control. A remarkable change in brashness of the treated wool was noted. The South American wool, which formerly was soft and appeared obviously unsuitable for pile fabrics, now was found to be brasher than the control.

45 The wool was then further processed, spun into yarn, dyed, and made into pile fabric.

The treated wool in the pile of the pile fabric was found upon test to have the stiffness and resilience characteristics required for carpet wool or other pile fabric wool, quite unlike the characteristics of the untreated wool, and quite unlike the characteristics of wool treated with silica soils by prior art methods.

50 A sample of the treated wool was brought to a boil in water over a period of 35 minutes and then 65 boiled for 40 minutes. The sample was subsequently dried and exposed to the air of the room for a sufficient time to bring it to equilibrium as to temperature and moisture content with the warehouse. It was found by comparison with a treated sample which had not undergone boiling, that the brashness imparted by the treatment was substantially retained during the boiling. Similar experiments were made to determine the effect on the brashness of normal wool treatments 70 such as further processing, dusting, spinning,

weaving and laundering, and it was found that the brashness is retained with very slight loss during such further treatments.

*Example II*

The treatment above referred to in Example I was applied to a dyed carpet wool blend containing small quantities of wool of inferior brashness, retaining a sample of the same blend untreated as a control. The treated sample and the control were then spun into carpet yarn and woven into velvet carpet, after which both samples were tested by U. S. Testing Company on the National Bureau of Standards carpet wear tester. The pile in each case was worn down to  $\frac{1}{4}$  of the net crushed pile height under the standard procedure, operating at 72° F. and 65% relative humidity. Figure 2 illustrates the best results, plotting net pile height in thousandths of an inch as ordinate and revolutions of tester, undergone by sample as abscissae. Curve 1 is for the treated sample and curve 2 is for the control. This shows that the sample of the untreated carpet wool blend withstood 120,000 revolutions to failure while the sample of the same wool blend treated according to the invention withstood 300,000 revolutions to failure or an improvement of 130% in wear resistance. In every other respect which could be determined by observation and tests applied, the treated sample was equal to or superior to the untreated sample. The treated sample exhibited enhanced brashness and the improvement in brashness of the treated sample is believed to be responsible for the improved wear resistance. A 50 hour fadeometer test showed no unfavorable effect on the dyeing when the carpet made from the treated wool was compared with the control.

*Example III*

The procedure of Example I was followed, using 0.05% sulphuric acid. The brashness imparted was less pronounced, but otherwise the results were comparable to those of Example I. The brashness was largely retained after 20 minutes boiling.

*Example IV*

The procedure of Example I was followed except that hydrogen peroxide was added to the solution in a concentration of two volume strengths. The solution performed the functions of the bleach normally used besides applying the treatment in accordance with the invention. The product was from the standpoint of the invention identical with that of Example I.

*Example V*

A series of experiments were carried out using various concentrations of acids. It was found that as the acid concentration increased, the tendency to agglomerate the silica particles increased, and when the pH reached the acid side of 2, the dusting of particles deposited on the surface became prohibitive in further processing. Thus beyond this pH value the desirable effect on the brashness of the fiber is clouded by the undesirable tendency to form surface deposit. It was found by this series of experiments that the desirable brashness can be obtained using a pH range in the bath between 2 and 6, but pH ranges on the acid side of 2 are not practical because of eventual excessive agglomeration in the continuous processing, and pH ranges on the alkaline side of 6 do not give satisfactory improvement in brashness or permanence in deposit unless the technique of acidifying the wool itself is

used as referred to below. Best results from the standpoint of improvements in the characteristics associated with brashness and elimination of dusting are obtained using pH ranges between 3 and 5.

*Example VI*

Using the procedure of Example I and the pH ranges of Example V, alkaline scoured wool was treated after having been first acidified to various pH's on the wool. It was found that the treatment would proceed satisfactorily even though the resultant wool was alkaline to a pH as high as 8, but that desirable results were not obtained when the pH on the wool was on the alkaline side of 8. In determining the pH on the wool, the procedure used was to dilute five grams of dry wool with 150 milliliters of distilled water, which had been boiled to expel carbon dioxide. The wool is placed in the boiling water and agitated during cooling of the water to room temperature, after which the pH of the solution is taken as the pH on the wool.

*Example VII*

The procedure of Example I was repeated, adding a dispersing agent to maintain the dispersion of the silica in the presence of impurities brought in by the wool. The dispersing agent used was an alkyl naphthalene sodium sulphonate, methyl naphthalene sodium sulphonate in a concentration of 0.1%. It was found that the dispersing agent made it possible to operate for a longer period without dropping the bath, and reduced the tendency to form precipitate.

The alkyl naphthalene sodium sulphonates generally are suitable. Other dispersing agents were used successfully, including sodium hexametaphosphate, tetrasodium pyrophosphate, sodium tetraphosphate, naphthalene sulphonic acid condensed with formaldehyde, and naphthalene sulphonic acid derivatives condensed with formaldehyde. It was found that any water soluble dispersing agent might be used and that the aromatic sulphonates and aromatic sulphonic acids were most suitable. The concentration of dispersing agent may vary from 0.01 to 1%.

*Example VIII*

The procedure of Example I was repeated with the addition of a dispersing agent as in Example VII followed by the addition of 0.1% of a substantive agent. Suitable substantive agents are quaternary ammonium salts, such as aliphatic-aromatic quaternary ammonium halides, examples of which are trialkyl benzyl ammonium chloride, as for example trimethyl benzyl ammonium chloride, triethyl benzyl ammonium chloride, dimethyl ethyl benzyl ammonium chloride, diethyl methyl benzyl ammonium chloride, benzyl cetyl dimethyl ammonium chloride and benzyl cetyl diethyl ammonium chloride; also tetra alkyl quaternary ammonium halides such as trimethyl cetyl quaternary ammonium chloride, triethyl cetyl quaternary ammonium chloride. The concentration of substantive agent may vary from 0.01 to 1%. In the case of substantive agents, there is a tendency to exhaust the bath, and such exhaustion must be made up by controlled additions of silica sol to the bath, and limiting the time of treatment in accordance with the desired pick-up. There is a further tendency to induce undesirable precipitation which should be inhibited by the use of increased quantities of dispersing agent.

Additional experiments indicated that any other suitable acid can be used instead of sul-

phuric acid, results identical with those set forth in Example I having been obtained with other acids when the pH was the same. The invention is capable of operation with hydrochloric acid, oxalic acid, citric acid, phosphoric acid or any other suitable acid.

The concentration of silica sol in the bath may vary from 0.3% to 5%, and the pick-up of silica may vary from 0.1% to 2% on the weight of the dry wool.

In the absence of a substantive agent, the time of exposure is not critical as long as the wool is thoroughly wet by the treating bath. For good results in continuous treatment it is not wise to use an exposure time of less than one-half minute and the usual exposure time is about one and one-half minutes, but in the absence of substantive the time may be extended indefinitely as desired. Where batch treatment is used in an open tank, dyeing machine or the like, the time will vary to suit the particular equipment.

The temperature used may vary from the ambient up to close to a boil, although a temperature in excess of about 125° F. is not desirable as it is unduly destructive of the sol. The treating solution has a wide degree of compatibility. As pointed out a bleaching agent such as hydrogen peroxide (suitable in a concentration of 1 to 3 volume strengths) may operate in the same bath. Likewise the treatment of the invention may be applied before or after dyeing or in the presence of a dye bath.

#### Example IX

The procedure of Example VIII was carried out, including 2% of polystyrene emulsion in the bath. The resin concentration may vary from 0.1 to 5% of the bath. It was found that the process of the invention was carried out without interference with the resin treatment. Water dispersions of other synthetic resins may be used in the treating bath, typical examples being acrylic, phenol-formaldehyde and melamine, in such form as to be stable in the desired pH range. Oil emulsions should however be avoided.

#### Example X

Instead of using a treating solution within the acid range specified, acidity may be imparted to the wool. The procedure of Example I was followed, with the additional step of acidifying the wool by treatment with 0.1% sulphuric acid subsequent to the degreasing and prior to the exposure to the silica sol. The silica sol was maintained at pH 7, omitting the sulphuric acid in the silica sol solution. The exposure time was limited so that the pH of the wool at the time it was extracted and removed from the treating bath was on the acid side of 7. The results obtained were comparable to those secured in Example I, but the treatment was more critical in that the exposure time required careful regulation. Where reliance is placed on acidulating the wool, the pH of the wool at the time it enters the solution of silica sol should be between 2 and 6. The pH of the solution may in this case vary between 6 and 8, and the pH on the wool at the time it leaves the treating solution should be on the acid side of 7. It will be observed, of course, that if the pH of the silica sol solution is between 2 and 6 rather than between 6 and 8, the operation is effectively the same as that of Example I.

#### Example XI

The procedure of Example II was applied to dyed carpet wool blend using spraying of the

treating solution followed by drying, instead of immersion in a liquid bath as in the procedure of Example II. The results were less uniform than those obtained in Example II but were otherwise generally similar. There was a much more pronounced surface deposit and more dusting present in the case of application by spraying than was characteristic of the immersion treatment. The permanence of the treatment was also inferior to that obtained by immersion and for this reason the spray treatment is not regarded as preferable.

In ordinary practice the wool, after drying and reaching equilibrium at room temperature will have a moisture content of the order of 12%.

It should be emphasized that the improvement in the characteristics associated with brashness produced by the invention will usually not be obvious while the wool is moist, but will in most cases only be recognizable when the wool has reached an equilibrium moisture content comparable to that encountered in normal warehouse storage.

The improvement in the characteristics associated with brashness of the wool is carried through from the fiber to the yarn and from the yarn to the fabric, and is particularly noticeable in improved wear and superior stiffness combined with resilience in a pile of a pile fabric. Figure 1 illustrates a pile fabric having a backing 20 and pile yarn 21 which has been treated in accordance with the invention. The pile yarn 21 will, in the normal case, have no measurable increase in diameter due to the treatment, but will definitely be improved in characteristics associated with brashness, particularly in the combination of resilience and stiffness sometimes called wiriness, and in remarkable increase in wear resistance. Thus the pile remains upstanding longer and will wear away more slowly than similar wool pile not having this treatment. Likewise the pile is desirably delustered by the treatment. The cost of the pile is considerably decreased, since the cost of soft wools such as South American blanket and clothing wools is generally less than that of high grade carpet wools.

The pile 21 has the remarkable property of retaining its improved characteristics notwithstanding usual treatments such as laundering, and even after several hours of boiling. Dyeing can be applied to the fabric without loss of the improved properties.

In essence my experiments indicate that a matrix or network of silica is introduced to the fibers of the pile 21 which appears to combine chemically, apparently due to secondary valence. It would appear that under the influence of the acid the silica sol is caused to agglomerate and produce gross aggregates which enter the fiber and stiffen and increase its wear resistance. In the process of formation and entry into the fiber it would appear that the sol converts to gel, at least in part, and that the gel contributes to obtaining the unusual properties. This conclusion is confirmed by the fact that under normal operating conditions a small amount of silica precipitates from the treating bath, apparently due to greatly excessive agglomeration.

The extent of agglomeration can be controlled by varying the silica concentration of the solution and more especially by varying the acidity. The greater the acidity, the more pronounced the tendency to agglomerate and the greater the concentration of silica the greater the tendency

to agglomerate. The wasteful precipitate can be retarded by the presence of a suitable dispersing agent, as mentioned, and where a considerable amount of foreign matter from the wool is being carried into the treating bath, the presence of a dispersing agent is very desirable to suppress the tendency of the impurities to throw down the sol and shorten the life of the bath.

Oil emulsion should be avoided and it is very undesirable to attempt to apply the present invention in a bath where oil emulsion is being used, as in the picker where silica sol has previously been employed.

Providing the above precautions are followed, results can be obtained reliably without undue waste of chemicals.

When reference is made to imparting the characteristics associated with brashness, it will be understood that such characteristics may be either created or enhanced.

In view of my invention and disclosure variations and modifications to meet individual whim or particular need will doubtless become evident to others skilled in the art, to obtain all or part of the benefits of my invention without copying the process and product shown, and I, therefore, claim all such insofar as they fall within the reasonable spirit and scope of my claims.

Having thus described my invention what I claim as new and desire to secure by Letters Patent is:

1. The process of treating wool to impart characteristics associated with brashness, which comprises degreasing the wool to a total grease content of less than  $\frac{3}{4}\%$  based on the dry weight of the fiber, subsequently treating the wool at any stage in its processing with a solution consisting of an acidified aqueous dispersion of colloidal silica of an initial silica particle size between 10 and 100 millimicrons and having a pH of 2 to 6 until the pick-up of silica by the wool is in the range between 0.1 and 2% based on the dry weight of the fiber, and drying the wool.

2. The method of increasing the wear resistance of wool for pile fabrics, which comprises degreasing the wool to a total grease content of less than  $\frac{3}{4}\%$  based on the dry weight of the fiber, subsequently treating the wool with a solution consisting of an acidified aqueous dispersion of colloidal silica of an initial silica particle size between 10 and 100 millimicrons having a pH of 2 to 6 until the pick-up of silica by the wool is in the range between 0.1 and 2% based on the dry weight of the fiber, thereby agglomerating the silica and forming gel in the solution, and then allowing the wool to dry.

3. The process of imparting to wool the characteristics associated with brashness, which comprises degreasing the wool to a total grease content of less than  $\frac{3}{4}\%$  based on the dry weight of the fiber, treating the wool in a solution consisting of an acidified aqueous dispersion of colloidal silica of an initial silica particle size between 10 and 100 millimicrons and having a pH of 2 to 6 in the presence of gross agglomerates of silica formed under the influence of the acid until the pick-up is in the range from 0.1 to 2% silica based on the dry weight of the fiber, and then drying the wool.

4. The process of treating wool, which comprises degreasing the wool to a total grease content of less than  $\frac{3}{4}\%$  based on the dry weight of

the fiber, treating the wool in a solution consisting of an acidified aqueous dispersion of colloidal silica having a pH of 2 to 6 of an initial silica particle size between 10 and 100 millimicrons and having a pH of 2 to 6 in the presence of a dispersing agent and a substantive agent until the pick-up of silica by the wool is in the range between 0.1 and 2% based on the dry weight of the fiber, and drying the treated wool.

5. The process of treating wool to impart characteristics associated with brashness, which comprises degreasing the wool to a total grease content below  $\frac{3}{4}\%$  based on the dry weight of the fiber, treating the wool in a solution consisting of an acidified aqueous dispersion of colloidal silica of an initial silica particle size between 10 and 100 millimicrons having a pH of 2 to 6 and containing gross aggregates of colloidal silica until the pick-up of silica by the wool is in the range between 0.1 and 2% based on the dry weight of the fiber, and drying the wool.

6. The process of treating wool to impart characteristics associated with brashness, which comprises degreasing the wool to a total grease content below  $\frac{3}{4}\%$  based on the dry weight of the fiber, acidifying the wool to a pH on the wool of 2 to 6, and treating the wool with a solution consisting of an aqueous dispersion of colloidal silica of an initial silica particle size between 10 and 100 millimicrons, at a pH of 6 to 8 until the pH on the wool has increased to a value toward the alkaline side of its original pH but still on the acid side of neutral until the pick-up of silica by the wool is in the range between 0.1 and 2% based on the dry weight of the fiber, and drying the wool.

7. A wood pile fabric in which the wool fibers have a silica matrix imparted by degreasing the wool to a total grease content of less than  $\frac{3}{4}\%$  based on the dry weight of the wool, treating the wool with a solution consisting of an acidified aqueous dispersion of colloidal silica of an initial silica particle size between 10 and 100 millimicrons and having a pH of 2 to 6 until the wool has picked up from 0.1 to 2% of silica based on the dry weight of the wool, and drying the wool.

8. A wood pile fabric in which the wool fibers of the pile have a silica matrix imparted by degreasing the wool to a total grease content of less than  $\frac{3}{4}\%$  based on the dry weight of the fiber, acidifying the wool to a pH on the wool of 2 to 6 and treating the wool with an acidified aqueous dispersion of colloidal silica of an initial silica particle size between 10 and 100 millimicrons having a pH of 6 to 8, until the pH on the wool has changed toward the alkaline side but is still on the acid side of neutral and until the pick-up of silica by the wool is in the range between 0.1 and 2% based on the dry weight of the fiber, and then drying the wool.

JACKSON BAUER.

#### REFERENCES CITED

The following references are of record in the file of this patent:

#### UNITED STATES PATENTS

| Number    | Name          | Date          |
|-----------|---------------|---------------|
| 1,629,241 | Ubbelohoe     | May 17, 1927  |
| 1,961,863 | Parker        | June 5, 1934  |
| 2,201,891 | Edgar et al.  | May 21, 1940  |
| 2,327,278 | Lurie         | Aug. 17, 1943 |
| 2,443,512 | Powers et al. | June 15, 1948 |